

J. H. YOUNG.  
PROTECTED METAL ARTICLE.  
APPLICATION FILED FEB. 27, 1920.

1,366,999.

Patented Feb. 1, 1921.

Fig. 1.



Anti-stick Materi  
d - Hard Asphalt.  
c - Soft Asphalt.  
b - Metal.

Fig. 2.

Inventor:  
James Howard Young  
by Jas. H. Churchill, atty.

# UNITED STATES PATENT OFFICE.

JAMES HOWARD YOUNG, OF PITTSBURGH, PENNSYLVANIA, ASSIGNOR TO H. H. ROBERTSON CO., OF PITTSBURGH, PENNSYLVANIA, A CORPORATION OF PENNSYLVANIA.

## PROTECTED METAL ARTICLE.

1,366,999.

Specification of Letters Patent.

Patented Feb. 1, 1921.

Application filed February 27, 1920. Serial No. 361,725.

To all whom it may concern:

Be it known that I, JAMES HOWARD YOUNG, a citizen of the United States, residing in Pittsburgh, county of Allegheny, and State of Pennsylvania, have invented an Improvement in Protected Metal Articles, of which the following description, in connection with the accompanying drawings, is a specification, like letters on the drawings representing like parts.

This invention relates to a protected metal article particularly adapted for building purposes and which will be hereinafter referred to as a protected metal sheet.

The invention has for its object to provide a protected metal sheet, which is capable of resisting weather conditions and acid and alkaline fumes, and which can be produced at such low cost as to enable it to be used in those places where heretofore only galvanized iron was available on account of the cost.

To this end, the metal sheet is provided, preferably on all of its surfaces and edges, with a coating composed of a layer of relatively low melting point asphalt, which will be hereinafter referred to as a soft asphalt, which is applied to the steel or other metal sheet, and a second layer of relatively high melting point asphalt, which will be hereinafter referred to as hard asphalt, is applied to the first layer and bonds therewith.

The coated metal sheet may and preferably will be provided with an exterior layer of anti-stick material.

The particular features of the invention will be pointed out in the claims at the end of this specification.

Figure 1 is a plan of a portion of a protected metal sheet embodying this invention, and

Fig. 2, a cross section on the line 2—2, Fig. 1.

Referring to the drawings, *a* represents a metal sheet or other article, which is cleaned in the usual manner and has applied to it a soft asphalt or bituminous material of relatively low melting point to form a layer *b* of substantial thickness.

The layer *b* may be formed on the metal sheet *a* by passing the latter through a bath of melted asphalt or between rolls supplied with hot asphalt in a manner well understood.

After the layer *b* of soft asphalt has been formed on the metal sheet *a*, a second layer *c* of relatively hard asphalt or like bituminous material of relatively high melting point is applied to the layer *b* while the latter is in more or less tacky condition, so that the second layer *c* will bond or unite with the first layer *b*.

The protected metal sheet thus produced, is especially advantageous for building purposes, as the metal sheet is effectively protected against the action of the weather and acid and alkali fumes by the two layers of asphalt and particularly by the layer *b* of soft asphalt, while the layer *c* of relatively hard asphalt protects the layer *b* and is of sufficient hardness to enable the coated sheet to be handled and worked in the warm temperatures of the summer.

By the mixing of the outer surface of the layer *b* with the inner surface of the layer *c*, the two asphalt layers are directly bonded together so that one modifies the other to such extent as to form a protective coating capable of resisting relatively wide changes in temperature, whereby the coating under the high temperatures of the summer months retains its hardness sufficiently to be handled, and under the low temperatures of the winter months retains sufficient ductility to avoid becoming brittle and cracked.

These advantageous features enable the protected metal sheet to be manufactured and used all the year around, and bent or otherwise manipulated without injuring the protective coating.

Furthermore the protected metal sheet can be produced at a less cost than galvanized iron and consequently can be used where the latter only is now available on account of cost, and it is superior to galvanized iron as the latter is attacked readily by acid fumes.

The protected metal sheet may and preferably will be provided with a relatively thin layer or film *d* of anti-stick material, 100 preferably that described in United States Patent No. 1,327,933 granted to me January 13, 1920, which mentions viscose and a soluble soapy material incorporated therewith.

## Claims.

1. As an improved article of manufacture, a metal article provided with a protective coating, comprising a layer of bituminous

material of relatively low melting point affixed directly to the metal article, and a second layer of bituminous material of relatively higher melting point applied directly

5. to and united with the first-mentioned layer.

2. As an improved article of manufacture, a metal article provided with a protective coating, comprising a layer of relatively soft asphalt affixed to the metal article, and 10 a layer of relatively harder asphalt applied directly to and united with said relatively soft asphalt layer.

3. As an improved article of manufacture, a metal article provided with a protective 15 coating, comprising a layer of relatively soft asphalt affixed to the metal article, a layer of relatively harder asphalt applied di-

rectly to and united with said relatively soft asphalt layer, and a film of anti-stick material covering the relatively harder asphalt 20 layer.

4. As an improved article of manufacture, a metal article enveloped by a weather and acid resisting coating composed of a layer of material capable of resisting relatively 25 high temperatures, and a layer of material capable of resisting relatively low temperatures, said latter layer being applied directly to said metal article and being directly bonded with the first-mentioned layer. 30

In testimony whereof I have signed my name to this specification.

JAMES HOWARD YOUNG.